

May 1, 1923.

H. T. YARYAN

1,453,303

PROCESS OF MANUFACTURING PLATES FOR ARTIFICIAL DENTURES

Filed Sept. 23, 1921



Fig. 1.



Fig. 2.



Fig. 3.



Fig. 4.



Fig. 5.

INVENTOR.

Homer T. Yaryan,  
By *Cornell & Crampton*,  
Atty.

## UNITED STATES PATENT OFFICE.

HOMER T. YARYAN, OF ST. PETERSBURG, FLORIDA.

## PROCESS OF MANUFACTURING PLATES FOR ARTIFICIAL DENTURES.

Application filed September 28, 1921. Serial No. 502,639.

*To all whom it may concern:*

Be it known that I, HOMER T. YARYAN, a citizen of the United States, and a resident of St. Petersburg, county of Pinellas, and State of Florida, have made an invention appertaining to Processes of Manufacturing Plates for Artificial Dentures; and I do hereby declare the following to be a full, clear, and exact description of the invention, such as will enable others skilled in the art to which it appertains to make and use the same, reference being had to the accompanying drawings, and to the characters of reference marked thereon, which form a part of this specification.

This invention relates to the manufacture of artificial dentures, and particularly to those composed of metal.

Artificial dentures are more generally made of either gold or vulcanite, the latter being the more common. Gold plates or dentures are made either by what is known as the swaging method or by casting, both of which have their disadvantages. In making a denture by the swaging method a sheet of gold of the proper thickness is thoroughly annealed, and from an impression taken from the mouth a reverse cast is made, and between the two dies thus formed the gold sheet after annealing is hammered to cause it to assume the irregularities of the dies. The dies, however, soon become battered and new dies are then made and the annealing of the gold and the hammering is repeated as before until what is considered as a good plate is produced. Some times as many as three and four sets of dies are used in the making of a plate. The result is an imperfectly fitting plate. As attachments for holding the vulcanite must be soldered on to the gold at a high temperature it is thereby so annealed that it is liable to get out of shape in use or handling. For these reasons the casting process is at present the most popular of the two. In making plates or dentures by the casting method considerable shrinkage takes place in the metal when cooling so that only an approximate fit to the mouth can be obtained. The disadvantages of both the swaging and casting processes are that plates made therefrom badly fit the mouth, and secondly, that they are extremely expensive and therefore rarely used until the gums have become hardened.

On account of this expense, plates made by

the vulcanized rubber process are customarily used for temporary sets.

In making a plate by the vulcanizing process, the vulcanizing of the vulcanite causes it to shrink approximately 10%, and therefore a plate made by this process which would otherwise have been correct is distorted to the extent of such shrinkage. If the tissues are soft they will in many cases adapt themselves to this distorted impression of the mouth, but if they are hard tissues which will not yield, irritation takes place and it is necessary to grind and cut and fit the plate until made bearable to the wearer. Another objection to the vulcanite plate is that it is a very poor conductor of heat and prevents the proper radiation of heat from the mucous membrane over which it is placed, thereby leading to excessive re-absorption of the hard tissues and a lowering of the vitality of the soft tissues in consequence of which they are more subject to irritation.

The object of my invention is to make an artificial metal denture which is a perfect fit of the portion of the mouth to which it is to be applied, and which contains a small percentage of precious metal as compared with gold or other precious metal dentures as now made, and which also affords a ready conductor for heat, thereby producing a more efficient and cheaper artificial denture than, to my knowledge, has heretofore been produced, and also producing a healthy condition of the gums and tissues of the mouth when such dentures are worn.

Other objects and advantages of the invention will be apparent from the following detailed description.

While the invention is capable of being practiced in different ways, a preferred method of practicing the same is illustrated in the accompanying drawings, in which,—

Figure 1 is a view of an impression formed by the first step. Fig. 2 is a view of a cast formed by the second step. Fig. 3 is an illustration of the step for electrically depositing a plate of metal on a portion of the cast. Fig. 4 is a view of the electro-plate with the anchoring attachments thereon for the gum forming vulcanite, and Fig. 5 illustrates the electro-plating step by which gold or silver may be deposited on the plate.

In practicing my method of producing

artificial dentures, a negative impression, such as shown in Fig. 1, of wax or other suitable material is first taken of the mouth and from this is preferably made a plastic 5 cast or negative such as shown in Fig. 2. A plate blank of suitable base metal, for instance copper, is then deposited electrically on the cast by the art known as electrotyping or galvanoplasty the cast having been first "stopped off" with varnish or 10 other suitable material to limit the surface of the cast on which the electrical deposit is to be made. The cast is left in the electrotyping bath until a plate of desired thickness has been formed, after which the plate 15 is removed from the cast and the side thereof which is opposed to the cast is then dressed to render it smooth, while the side thereof next to the cast is left as formed, 20 it being perfectly smooth and requiring no dressing or polishing. In dressing the cast, however, it is preferable to leave rough the portion thereof which is to be covered by the vulcanite intended to represent the gums 25 and to carry the teeth, as this rough condition is an advantage in securely anchoring the vulcanite to the plate. Only that portion of the plate which the tongue and food touches is dressed and polished to present 30 a perfectly smooth surface.

After the dressing operation, devices called attachments are soldered at spaced points to the plate, the soldering being only sufficient to temporarily hold the "attachments" in position. The attachment which 35 usually comprises a wire bent in various shapes serves as an anchoring means for the vulcanite, which is later secured to the plate to represent the gum. The plate is 40 then returned to the electrotyping bath after having first been stepped off with varnish or other suitable material on that portion thereof which comes in contact with the gums and roof of the mouth, so that the 45 electrical deposit will take place only on the portion of the plate to which the attachment is secured. The plate is left in the bath until sufficient copper or other metal has been deposited thereon to cover all the 50 soldered spots and also to imbed the wire attachments and make them a part of the plate. The plate is then polished to render smooth that portion thereof coming in contact with the tongue.

55 The next step preferably consists of depositing a moderate thickness of silver on the plate blank by silver plating and then subjecting the plate to a gold plating step. The gold coating is only of sufficient thickness 60 to provide a thin coating thereon, as the portion thereof to which the vulcanite is to be secured and the surface in contact with the roof of the mouth requires only a thin coat. These portions are then 65 "stopped off" and that portion of the plate

which is subjected to wear is given an extra heavy coating of gold. This having been done the plate is ready for the dentist to attach the gums and teeth in any suitable way. The silver plating of the plate 70 is done merely as a precautionary measure so that if the gold coating wears off in use the white coating of silver will show and indicate that the plate should be again coated with gold. While it is preferable 75 to deposit the gold on a silver coating, the gold or other suitable metal forming the exterior coating of the plate may be deposited directly on the copper or other metal comprising the blank and formed by the 80 electrotyping step.

The advantages of my method of making artificial dentures, among others, are first, the production of a plate which perfectly 85 fits the mouth provided the impression taken of the mouth is correct; second, the use of a very small percentage of precious metal as compared with gold dentures as now made, a first-class plate made by my method requiring about  $\frac{1}{4}$  of the gold used 90 in making a gold plate by the methods heretofore employed; third, the gold is deposited exactly where it is needed and in sufficient quantity to resist wear; fourth, the plate on account of its thinness 95 conducts heat readily and therefore produces a healthy condition of the gums and tissues of the mouth; fifth, the ease with which the gold may be replaced by replating when wear occurs; and sixth, a plate produced by 100 my method while strong and rigid, is of considerably less weight than a gold plate, thereby lending to the ease and comfort of the wearer of the same.

It is evident that the plate formed by the electrotyping process may be of any thickness desired depending on the weight or strength of the denture desired, and that the 105 coatings of silver and gold may also be of a thickness desired depending largely on the expense which the patient wishes to put in the plate.

While I have particularly described the 110 making of the electrotyping blank from a positive cast or reproduction of the mouth, it might be made from the negative impression or reproduction but this would not be desirable, for with the latter the rough or outer side of the blank deposit would constitute the side thereof intended to have contact with the roof of the mouth and it would therefore be necessary to grind and polish and shape this side to conform to the mouth so that the plate is firmly held to position when placed in the mouth. If the deposit 115 from the blank plate is made on a positive reproduction of the mouth, the side of the blank which is to fit against the roof of the mouth is perfectly formed to conform to the shape and irregularities of the roof so that 120 125 130

no subsequent shaping of that side of the blank is required.

I have particularly described my method with reference to depositing copper or other 5 cheaper metal on the reproduction of the mouth and then plating the blank with gold, as this is the preferable method of practicing the invention. It is not desired, however, to restrict the protection afforded 10 hereby to this particular method as it is known that gold may be directly deposited on the reproduction of the mouth by the electrotyping or galvanoplasty method and the vulcanite anchoring attachments secured 15 to the gold blank, after which the blank may again be placed in the bath to coat the attachments and unite them closely with the blank.

I wish it understood that my invention is 20 not limited to any specific means or method of practicing the same, except in so far as it is limited by the claims.

Having thus described my invention, what I claim as new and desire to secure by Letters Patent, is,—

1. The process of manufacturing plates for artificial dentures, which consists in taking a reproduction of the mouth, electrically depositing a base metal on the reproduction to form a plate blank, attaching a vulcanite anchoring means to the blank, and plating the blank with a metal which is non-corrosive and not objectionable to the mouth.

2. The process of manufacturing plates for artificial dentures, which consists in taking a reproduction of the mouth, forming a metal plate blank on the reproduction by the art of galvanoplasty, tacking a vulcanite anchoring attachment to the blank, then again subjecting the blank to the electroplating process to securely unite the attachment to the blank and then plating the blank

with a metal which is noncorrosive and not objectionable to the mouth.

3. The process of manufacturing plates 45 for artificial dentures, which consists in taking a correct impression of the mouth, forming a cast from the impression, electrically depositing copper on the cast to form a blank of the plate thereon, soldering vulcanite anchoring means to the blank, then again subjecting the blank to an electrical deposit of metal to closely unite the blank and anchoring means, then coating the blank 50 with a metal which is noncorrosive and not 55 objectionable to the mouth.

4. The process of manufacturing plates for artificial dentures, which consists in taking a correct impression of the mouth, forming a cast from the impression, electrically 60 depositing copper on the cast to form a blank of the plate thereon, soldering vulcanite anchoring means to the blank, then again subjecting the blank to an electrical deposit of metal to closely unite the 65 blank and anchoring means, and then successively coating the blank with a suitable metal of a color other than gold and with gold.

5. The process of manufacturing plates for artificial dentures, which consists in 70 taking a reproduction of a portion of the mouth, electrically depositing a metal on the reproduction to form a blank, attaching a vulcanite anchoring means to the blank, then again subjecting the blank to an electrical 75 deposit of metal to closely unite the blank and anchoring means having first dressed the portion of the blank to smooth a part at least of the surface thereof on which the deposit takes place.

In testimony whereof, I have hereunto signed my name to this specification.

HOMER T. YARYAN.